

Dec. 29, 1964

SATORU TAGUCHI ETAL  
METHOD FOR PRODUCING SILICON STEEL STRIPS  
HAVING CUBE-ON-FACE ORIENTATION

3,163,564

Filed July 9, 1962

3 Sheets-Sheet 1

FIG. 1



FIG. 2



The arrow shows the easy direction of magnetization

FIG. 3



INVENTORS

Satoru Taguchi  
Akira Sakakura  
Takashi Yasunari  
Henderoth, Lind & Bonack  
attorneys

BY

Dec. 29, 1964

SATORU TAGUCHI ET AL  
METHOD FOR PRODUCING SILICON STEEL STRIPS  
HAVING CUBE-ON-FACE ORIENTATION

3,163,564

Filed July 9, 1962

3 Sheets-Sheet 2

FIG. 4



FIG. 5



INVENTOR.  
Satoru Taguchi  
Akira Sakakura  
Takashi Yasunari  
BY  
Wenderoth, Lind & Ponack  
attorneys

Dec. 29, 1964

SATORU TAGUCHI ET AL  
METHOD FOR PRODUCING SILICON STEEL STRIPS  
HAVING CUBE-ON-FACE ORIENTATION

Filed July 9, 1962

3,163,564

3 Sheets-Sheet 3

FIG. 6



FIG. 7



FIG. 8



INVENTOR.

BY Satoru Taguchi  
Akira Sakakura  
Takashi Yasunari  
Stenderoth, Lund & Ponack  
Attorneys

1

3,163,564

## METHOD FOR PRODUCING SILICON STEEL STRIPS HAVING CUBE-ON-FACE ORIENTATION

Satoru Taguchi, Akira Sakakura, and Takashi Yasunari, Yawata, Japan, assignors to Yawata Iron and Steel Co., Ltd., Tokyo, Japan

Filed July 9, 1962, Ser. No. 288,277

Claims priority, application Japan, Mar. 18, 1958, 33/7,092; Oct. 8, 1958, 33/28,745

2 Claims. (Cl. 148—111)

This application is a continuation-in-part application of our co-pending applications Ser. No. 797,361, filed March 5, 1959, and Ser. No. 844,450, filed October 5, 1959.

The present invention relates to a method for producing a so-called double oriented magnetic silicon steel strip which has easy magnetization axes [001] in two right-angled directions in the rolling plane of the steel strip and in which a (001) plane appears in the rolling plane.

Hitherto, silicon steel sheets (and this term is used hereinafter to include steel strips) have been used as a soft magnetic material, for iron cores of transformer, electric generators and the like. Many attempts have been made to control the crystal orientations of such silicon steel sheets destined for the aforesaid uses in order to obtain sheets of oriented silicon steel having a cubic crystal structure, in which there exist 3 mutually-perpendicular directions of easy magnetization (directions of cube axes <100>), and, which results in the advantage that, when a magnetic field is applied parallel to any of these <100> directions, a minimum amount of energy is required to magnetize the silicon steel.

The first type of oriented silicon steel that satisfied such requirement was single-oriented silicon steel.

Single-oriented steel consists of cubes standing on edge, hence it is often referred to as having cube-on-edge orientation which is of the (110)[001] type, as illustrated in FIG. 1(a) of the accompanying drawings. The arrow indicates that easy magnetization is possible only along a single direction which is usually the direction of rolling. In fact, lines representing the other cube axis would extend out from the top and the bottom of the sheet at angles of 45°. Therefore, as is well known to those skilled in the art, the magnetic induction and other magnetic properties are outstanding in the rolling direction, i.e., the [100] direction. However, in any other direction, for example, the direction transverse to the rolling direction of the sheet, the magnetic properties are greatly inferior because of the magnetization is not parallel to the edge of the cubic crystal structure.

It has long been the desire of this art to produce double-oriented silicon steel sheets which have a cube-on-face orientation, i.e., (100)[001] type crystals as illustrated in FIG. 1(b) of the drawings. For if sheets of a cube-on-face or double oriented grain texture can be produced, the easy direction of magnetization will be parallel to the length, width and height of the sheet; then the magnetic properties of the sheet would be outstanding both in the rolling direction of the sheet and in the transverse directions, i.e., the directions perpendicular to the rolling directions and to each other, in the sheet.

An object of this invention is to provide a process for producing double oriented silicon steel consisting substantially of a cube-on-face crystal, i.e., a (100)[001] type crystal and having consequently excellent magnetic characteristics along the two transverse directions, from a hot-rolled steel plate prepared by subjecting to a conventional hot rolling a silicon steel body and which is produced by a conventional melting (steelmaking) method or casting method.

A further object of this invention is to provide a process for producing double oriented silicon steel by a heat-treatment in a usual industrial atmosphere.

A still further object of this invention is to provide a

2

process for producing double oriented silicon steel having a desired thickness greater than that of the known double-oriented sheets, which process can be carried out successfully in a conventional industrial atmosphere.

An additional object of this invention is to provide a process for producing double oriented silicon steel having excellent magnetic characteristics, particularly in a comparatively high magnetic field, along two directions, a finally rolled direction and a transverse direction perpendicular thereto.

For a better understanding of the nature and objects of the invention, reference should be had to the following detailed description and drawings, in which:

FIG. 1 shows the crystal orientations and easy magnetization directions of crystal grains constituting single oriented silicon steel (a) and double oriented silicon steel (b) and Wassermann type oriented silicon steel (c).

FIG. 2 shows views of iron cores for transformers punched from single oriented steel (a) and from double oriented steel (b).

FIG. 3 shows views of iron cores for rotors punched from single oriented steel (a) and from double oriented steel (b).

FIG. 4 shows the relation between the Al contents after hot rolling on the one hand, and the magnetic characteristics after final annealing (the magnetic induction  $B_{10}$  and the iron loss  $W_{15/50}$  in the two outstanding directions, i.e., the final rolling direction and the direction perpendicular to it), on the other hand, as a result of a process mode A described hereinafter.

FIG. 5 shows the relation between the Al content after hot rolling and the magnetic characteristics after final annealing (the magnetic induction  $B_{10}$  and the iron loss  $W_{15/50}$  in 2 directions, i.e., the final rolling direction and the direction perpendicular to it), as a result of a process mode B described hereinafter; six different hot rolled silicon steel materials (plate thickness: 2.0 mm.) having chemical analyses as indicated in Table 1 are cold rolled with a reduction of about 30% in the same direction as that of hot rolling, then cold rolled with a reduction of about 30% in a direction approximately at a right angle thereto, then annealed for a period of 5 hours at the maximum holding temperature at 1100°C., then again cold rolled with a reduction of 70% in the same direction as that of the second cold rolling, and thereafter finally annealed for a period of 15 hours at the temperature of 1150°C.

FIG. 6 is a graph with two curves showing the relationship between short time anneal temperature and core loss after final anneal of the magnetic material produced according to mode A of the process according to our invention.

FIG. 7 is a graph showing the effects of the temperature of an intermediate box anneal over the magnetic properties of the magnetic material produced by mode A of the process according to this invention, and will be described in detail hereinafter.

FIG. 8 is a graph showing the relationship between the magnetic induction and the cold rolling reduction of the magnetic material manufactured by mode A of the process according to this invention, and will also be described in detail hereinafter.

In FIGURES 4-8, a solid line plotting black circle  $\bullet$  shows an iron loss in the final cold-rolling direction, a solid line plotting circles  $\circ$  an iron loss in the direction perpendicular thereto, a dotted line plotting black triangles  $\blacktriangle$  a magnetic induction in the final cold-rolling direction and a dotted line plotting triangles  $\triangle$  a magnetic induction in the direction perpendicular thereto.

Referring now to FIG. 1, there are shown differences in crystal orientations between the double-oriented silicon steel sheet produced in accordance with this invention and a single-oriented silicon steel sheet which has been de-

veloped heretofore. It will also be clear from the drawings that, since a double oriented silicon steel sheet has good magnetic properties in two directions, i.e., the rolling direction and the direction perpendicular thereto, such a silicon steel sheet can be used to make therefrom iron cores for electric machines far more advantageously than it is possible when a conventional single-oriented silicon steel sheet is used. While, when punching an iron core for a transformer as shown in FIG. 2, the iron core must be made by combining four elements 1, 2, 3 and 4 which are punched separately in the case of using a single-oriented silicon steel sheet, the iron core can be made by only a single punching, when double-oriented silicon steel sheet is used. Also, when an iron core for a rotor as shown in FIG. 3 is punched from a single-oriented silicon steel sheet, the easy magnetization direction does not coincide with the direction of the magnetic field in the part of the teeth 7, which results in a reduced magnetic capacity of the rotor. On the other hand, the iron core punched from the double oriented silicon steel sheet has good magnetizability at full capacity, and therefore the weight of the iron core may be light.

For the above reasons, double-oriented silicon steel sheet offers considerable industrial advantages as compared with the conventional single-oriented silicon steel sheet, but special metallurgical processes are needed in order to produce the desired double orientation because the cube-on-face, i.e., the (100)[001] orientation is not the usual configuration found in silicon steel.

For example, according to the method represented by German Patent Auslegeschrift 1,029,845, used by Vacuum-schmelze Co., Germany, double-oriented silicon steel is produced by hot rolling a silicon steel ingot obtained by vacuum melting, subjecting the hot rolled steel to several stages of cold rolling and repeated intermediate heat-treatments and, after final gauge has been attained, annealing finally in an oxygen-free inert atmosphere of high purity. However, this method requires many stages of cold rollings and intermediate heat-treatments, and it is also necessary that the atmosphere should be substantially free from oxygen, moisture and other oxidizing agents, so that  $\text{SiO}_2$  (silica) will not be produced on the surface of the steel sheet during the annealing and, furthermore, in case  $\text{SiO}_2$  is formed, it can be reduced to Si during the annealing treatment. It is, however, extremely difficult to maintain such annealing condition, at least on an industrial scale. In addition, another important drawback of this known method resides in the fact that crystal grains having almost complete (100)[001] orientation are grown when the thickness of the final product is less than 0.1 mm., but that, when the final product is thicker than the said limit value, the parallel relation between the rolling direction and the [001] direction or between the direction perpendicular to the rolling direction and the [010] direction deteriorates considerably, and, therefore, crystal grains having complete (100)[001] are no longer obtained, which makes it extremely disadvantageous as a process for producing iron core materials for heavy electric machines in which an article having a thickness of about 0.3 mm. is most desirable.

On the other hand, a process is also known in which an ingot having a (100)[001] orientation is made by casting molten silicon steel by using a special apparatus and the ingot is hot-rolled, cold-rolled and heat-treated. However, it is difficult to produce such an oriented ingot industrially and even if such an oriented ingot is obtained, this creates difficult problems in hot-rolling techniques, since the ingot must not be reheated during hot rolling.

Under these circumstances, it will be clear that the production of double-oriented silicon steel is very difficult to realize particularly on an industrial scale. We have now succeeded in producing double-oriented silicon steel having excellent magnetic characteristics in two directions, the rolling direction and the direction perpendicular thereto, by an industrial process for producing double-oriented

silicon steel which requires only the conventional industrial apparatus and no special, unusual operational methods. In the process according to our invention, a silicon steel element containing a small amount of Al is made by a conventional steel making method, and the steel is subjected to a conventional hot rolling to obtain a hot-rolled sheet, which is then treated with a novel mode of cold rollings including a cross rolling and heat-treatments in a conventional industrial atmosphere.

Moreover, in the known processes for producing double-oriented silicon steel sheets, considerably high cost is involved in carrying out these conventional processes on an industrial scale, since the steel to be used must be of considerably high purity and must, therefore, be prepared in a vacuum melting furnace.

On the other hand, in the improved process of our invention, any conventional steel melting method can be used, any specific measures are completely unnecessary in the necessary hot-rolling work, and the heat-treatment in the process according to this invention can be carried out under conventional conditions without the necessity of providing any specifically prepared atmosphere.

Furthermore, since in the process according to the present invention, the crystal grain of (100)[001] orientation being the constituent element of the produced double oriented silicon steel sheet grows independently of the thickness of the sheet, double oriented silicon steel having any thickness desired as electromagnetic materials can be produced. Therefore, the process of this invention represents a marked improvement over the known processes for producing double-oriented silicon steel sheets in which only articles having very limited thickness have been produced.

The objects of the present invention, as stated above, can be achieved by hot rolling a silicon steel element containing small but critical amounts of Si and Al, and treating it by a process including a cross cold rolling and in this case, the process of this invention is based on a new phenomenon, namely that the crystal grain having a (100)[001] orientation grows only when the hot rolled sheet contains a critical amount of Al and is cross-rolled and heat-treated.

A cross-rolling process had been described by Wassermann and by Bitter. However, the industrial value of this process is limited because the product obtained by their process shows a crystal orientation of the constituent crystal grain of a (100)[011] type as shown in FIG. 1(c) of the drawings, and because, consequently, the easy magnetization axis appears in a direction at an angle of 45° with the rolling direction and in the direction perpendicular thereto.

In the process according to this invention, we have succeeded in producing a double-oriented silicon steel sheet by subjecting a hot-rolled sheet containing critical amounts of Si and Al to a cross-rolling treatment, thereby growing a crystal grain having a (100)[001] orientation. Our inventive process which includes the aforesaid cross rolling treatment can be carried out in two different modes of operation which are designated as a process A and a process B respectively hereinafter.

The silicon steel material (steel ingot) used as starting material in this invention is preferably produced by a melting method and must contain above 2, and, to be really satisfactory, about 2.5% and up to 4% of Si and above 0.010 and indeed from 0.014% up to 0.040% of Al when using process mode A, or above 0.010 to 0.050% and better, from 0.015 to 0.041% of Al, when using process mode B (all percentages are by weight). Other allowable impurities may be contained in the starting material just as in conventional single oriented silicon steel and no unconventional restrictions need be imposed as to these impurities, except the aforesaid limits for Al and Si.

More particularly, the Si and Al contents of the steel, after hot-rolling should be from 2.7 to 3.8% of Si and from 0.016 to 0.030% of Al.

A typical, non-limitative analysis of steel suitably for use as starting material in the process of the present invention, and yielding optional results is the following:

2.98 to 3.10% Si, 0.020% Al, 0.04% C, 0.10% Mn, 0.012% P, 0.015% S, 0.10% Cu, 0.005% Ti and the balance Fe.

In regard to the carbon content, carbon is not a limiting element in the composition of the material of the present invention. However, in the ordinary industrially obtained ingot, it is difficult to make the carbon content less than 0.02%. On the other hand, if the carbon content is more than 0.06%, it will be very difficult in decarburization to eliminate the detrimental effect of the residual carbon on the magnetic characteristics of the product. Therefore, a carbon content from 0.02 to 0.06% shall be adopted.

If the Si content is greater than 4%, the ingot becomes brittle when it is rolled, in particular, cold-rolled as will be stated later, which causes undesirable phenomena such as rupture and if the Si content is less than 2%, a ferrite-austenite transformation occurs during the annealing process which will be explained later, whereby the crystal orientation, the production of which is the object of this invention, disappears. Also, in general, if the content of Si is low, the electric resistance of the steel sheet is lowered, which results in increasing eddy-current loss and iron loss. Therefore, in this invention, the content of Si is limited to higher than 2.5% and up to 4%.

With regard to the content of Al, processes are known in which Al is added in order to improve the magnetic properties of unoriented silicon steel sheet. For example, in one known process, an aluminum-containing silicon steel strip is produced by forming an Al-containing silicon steel having a suitable composition (Si 1-5%, Al 0.010-1.00% and C 0.02%), rolling the steel into a steel strip and then annealing the steel strip continuously at a temperature of 1500° to 1750° F. in a decarburization atmosphere to reduce the content of C to lower than 0.02%. However, in this known process, Al is added, because it was observed that, when Al is present in silicon steel, the temperature for making metallographic changes necessary for obtaining the best electric property is apt to be lowered while the temperature at which the silicon steel develops a  $\gamma$  phase is apt to be raised. This is said to have the practical effect that carbon, which would be dissolved in the steel, if Al were absent, remains out of solution, when Al is present, and in this state, C is available for removal from the steel as carbon oxides gas. However, such silicon steel of low watt loss values fails to show an outstanding single or, two outstanding directions of permeability which would characterize oriented silicon steel.

Another known process conceives a treatment of silicon steel containing 1.9% of Si and 0.20% Al. However, the purpose of adding Al in this known process is to obtain a proper crystalline condition in producing electric silicon steel flat stock, the last-mentioned process, without incurring the risk of intersecting the  $\gamma$  loop in the higher carbon steels produced in the said known process.

The products of these known processes are thus concerned with non-oriented silicon steel sheets and their magnetic properties are inferior to the double oriented silicon steel sheets of the present invention. Furthermore, while the purpose of adding Al in the case of the non-oriented silicon steel sheets is to control the appearance of the  $\gamma$  phase, the  $\gamma$  phase would not appear anyhow in the process according to the present invention, even if no Al were present. Therefore, the purpose of adding Al in the present process has nothing to do with the purposes for which the same is added in the above-described processes.

Also, in the well known process for imparting to silicon steel sheet a (110)[001] texture, generally referred to as "Goss texture" (see Patent 1,965,559), no effect of an addition of Al as suggested in the case of non-oriented

silicon steel sheets has been disclosed as being of any advantage, and where, aluminum has been present in single-oriented steel, it was merely incidentally, but since then, its presence was never provided for intentionally. In fact, the presence of Al in magnetizable steel has usually been avoided as far as possible, since Al is apt to form oxides such as  $Al_2O_3$  and the like in steel, which are harmful to the magnetic characteristics of the steel; and therefore, except for an unavoidable presence of less than 0.01% Al, stemming from the starting materials from which the steel is made, any content of Al has been, in general, eliminated. In double-oriented silicon steel sheet, no such effects as were adscribed to the addition of Al in the case of non-oriented silicon steel sheets, was generally expected, and, therefore, efforts were usually made to maintain the Al content, if any, as low as possible.

Only very recently, Möbius has disclosed that steel which is to be given (100)[001] cube texture, not by cross rolling treatment (90°), but by an inclined-angle rolling (50° to 70°), must have, in the case of silicon iron alloys, a content of between 0.5 and 2.5% of Si, in the case of aluminum iron alloys, a content between 0.5 and 2.0% Al, and, in the case of silicon-aluminum iron alloys, the sum of the quantities of silicon and aluminum together should be between 0.5 and 2.5%.

In contrast thereto, it is a fundamental feature of the process according to our invention and indispensable for carrying out the process successfully that, after hot rolling, the silicon steel ingot used in our process has an Al content above 0.010 and up to 0.040%, when used in process mode A, or up to 0.050% if used in mode B. The presence of aluminum within the stated critical limits is desirable in the process according to this invention since the advantages attained by the addition of Al more than make up for the disadvantages stated above, subject to certain conditions which will be explained further hereinafter.

Aluminum can be present in silicon steel in two forms, namely as acid-insoluble Al and acid-soluble Al. The former consists mainly of  $Al_2O_3$  produced due to the strong affinity of Al to oxygen and since it is harmful to the magnetic properties of steel, its formation must be avoided as much as possible, in this invention also. However, due to the progress made in steel-making and melting techniques, it has become possible to reduce greatly the content of acid-insoluble Al, even if a large amount of Al is added, by operating carefully during the adding process. We have found that, when the content of total Al is kept within the limits of 0.010 to 0.050%, the content of acid-insoluble Al contained in it is in the order of 0.005% independently of the total content, provided that care is taken that a sufficient amount of nitrogen is available in the atmosphere which is in contact with the steel while the latter is being produced and processed.

The remaining part of Al, namely the acid-soluble Al is an important component of this invention and it consists of Al present in a solid solution in silicon steel and Al which is present as a nitride such as AlN, of which the ratio depends upon the contents of total Al in the silicon steel and thermal conditions, such as melting conditions, hot-rolling conditions and annealing conditions, the reaction equation being as follows:



65 wherein, [Al] and [N] are Al and N respectively present as solid solutions in the silicon steel and AlN is a nitride of Al formed in the silicon steel.

When studying the formation of AlN, we found that the amount of AlN deposited at hot rolling is influenced greatly by the total Al content and by the conditions for making ingots. For example, in the case of producing silicon steel ingots in a conventional open-hearth furnace or electric furnace, N is present in the steel, and if Al is also present in the steel, Al is deposited as AlN. On the

other hand, if specific melting apparatus, such as a vacuum melting furnace and the like, are used, N is absent from the steel, and in this case hardly any AlN is formed even if a considerable amount of Al is contained in the steel. In other words, unless such specific melting apparatus is used in the production of steel ingot, but the latter is produced by the common industrial techniques, and is hot-rolled, the acid-soluble Al present in the hot rolled product consists partly of AlN.

The AlN content should amount to at least 0.0029% and preferably at least 0.0043 to 0.0045 and may be as high as 0.0073% and higher, calculated on the weight of the hot-rolled silicon steel.

In order to produce double oriented silicon steel by the process according to this invention, it is therefore another indispensable condition that acid-soluble Al mainly consisting of AlN is present either in the hot-rolled steel sheet or, at the latest, in the steel sheet prior to cross cold-rolling. This can be achieved by casting silicon steel material containing the above-defined small, but critical, amounts of Si and Al by any conventional steel-making method and/or melting apparatus, which permits nitrogen to be present in the steel, i.e., either introduce the same, or maintain the same in solution in the steel in sufficient amounts that the major portion, preferably 60% and more, of the aluminum present in the steel exists in acid-soluble form and a substantial portion of the latter as aluminum nitride, and then subjecting it to a conventional hot-rolling. Therefore, this process is very easy to carry out on an industrial scale and very economical as compared with the melting method which has hitherto been used for producing double oriented silicon steel sheets.

Wiener teaches in the United States Patent 2,965,526 a process for producing a single-oriented silicon steel strip by cold-rolling and heat-treating a hot-rolled silicon steel containing in a range of 0.001 to 0.05% at least one substance of a group consisting of metal sulfides, oxides and nitrides.

The differences between it and the present invention shall be described more particularly. First of all, the object product of said U.S. Patent 2,965,526 is a single-oriented silicon steel sheet consisting of crystal grains of such (110)[001] orientation as is shown in (a) in FIGURE 1 and shows favorable magnetic characteristics in the rolling direction only, whereas that of the present invention is a double-oriented silicon steel sheet consisting of crystal grains of such (100)[001] orientation as is shown in (b) in FIGURE 1 and shows favorable mag-

netic characteristics in the two directions of the rolling direction and the direction at right angles thereto. How industrially significant this is, is as already shown with examples in FIGURES 2 and 3. Secondly, the starting material of said U.S. Patent 2,965,526 is a hot-rolled silicon steel containing about 2.2 to 5.25% Si, 0.001 to 0.05% of at least one substance of a group consisting of metal oxides, sulphides and nitrides and maximum of 0.02% C, the rest being iron, whereas that of the present invention is a hot-rolled silicon steel containing above 2.5 and up to 4.0% Si, 0.010 to 0.050% Al, the larger part of which must exist as acid-soluble aluminum consisting to a substantial portion of AlN, apart from the unavoidably present small amount of acid-insoluble aluminum, and carbon in the range of 0.02 to 0.06% and is evidently a material quite different from the above. Thirdly, the treating process of the U.S. Patent 2,965,526 is the two-step cold-rolling method developed by N. P. Goss, whereas that of the present invention is a two-step or three-step cold-rolling method including cross-rolling and is quite different from the above.

The two above-mentioned modes A and B of carrying out the process according to the invention in practice will now be described in detail.

#### PROCESS MODE A

Hot-rolled sheets, preferably in the form of strips of 1.6 mm. in thickness obtained by subjecting to a conventional hot rolling ingots containing the above-defined critical contents of Si and Al, that are produced by a conventional electric furnace steel-making process, permitting formation of aluminum nitride as described above, are used as starting material.

More particularly, FIG. 4 gives the curves showing the relationship between the aluminum content prior to final anneal, core loss after final anneal, and magnetic induction radius when various specimens of the aforesaid starting material designated as A, B, C, D and E with the composition shown in Table 1 below or similar compositions including varying contents of aluminum and silicon within the above-defined limits are subjected to hot rolling to a thickness of 1.6 mm., pickling to remove scale resulting therefrom, an initial cold rolling in one direction with a reduction of 60%, then a final cold rolling in a direction approximately at right angle thereto with a reduction of 50%, then a short time anneal for about four minutes at the temperature of 800° C., and lastly a final anneal for fifteen hours at the temperature of 1150° C.

Table 1  
ANALYSIS OF STEEL AND MAGNETIC PROPERTIES

| Specimen | Analysis, percent |      |           |                 |          |          | Magnetic Test (Epstein) |                    |                 |
|----------|-------------------|------|-----------|-----------------|----------|----------|-------------------------|--------------------|-----------------|
|          | C                 | Si   | Al in all | Acid-soluble Al | N in all | N as AlN | Core Loss               |                    | B <sub>10</sub> |
|          |                   |      |           |                 |          |          | W <sub>10/50</sub>      | W <sub>15/50</sub> |                 |
| A-----   | 0.04              | 3.06 | 0.005     | 0.002           | 0.0043   | 0.0010   | 0.67                    | 1.90               | 15,180          |
|          | 0.005             | 3.01 | 0.005     | 0.002           | 0.0050   | 0.0010   | 0.66                    | 1.83               | 15,270          |
| B-----   | 0.04              | 3.02 | 0.014     | 0.011           | 0.0089   | 0.0043   | 0.55                    | 1.31               | 17,780          |
|          | 0.007             | 3.02 | 0.014     | 0.010           | 0.0089   | 0.0045   | 0.58                    | 1.33               | 17,570          |
| C-----   | 0.04              | 2.98 | 0.019     | 0.015           | 0.0095   | 0.0061   | 0.44                    | 1.02               | 18,120          |
|          | 0.006             | 2.98 | 0.018     | 0.015           | 0.0097   | 0.0059   | 0.47                    | 1.08               | 17,980          |
| D-----   | 0.04              | 2.99 | 0.023     | 0.018           | 0.0090   | 0.0061   | 0.42                    | 0.98               | 18,430          |
|          | 0.006             | 3.01 | 0.024     | 0.017           | 0.0088   | 0.0061   | 0.46                    | 1.06               | 18,050          |
| E-----   | 0.04              | 3.10 | 0.040     | 0.033           | 0.0078   | 0.0070   | 0.59                    | 1.50               | 16,830          |
|          | 0.006             | 3.02 | 0.039     | 0.031           | 0.0071   | 0.0071   | 0.65                    | 1.77               | 18,200          |

Remarks:

1. W<sub>10/50</sub> watts × 10 kilogausses at a frequency of 50 c.p.s. Unit: watts per kilogram; W<sub>15/50</sub> watts 15 kilogausses at a frequency of 50 c.p.s. Unit: watts per kilogram.
2. B<sub>10</sub> magnetic induction at 10 oersteds. Unit: Gauss.
3. Referring to Magnetic Test Value (Epstein), upper value refers to that of final rolling direction while the lower that of the direction right angle thereto. Magnetic value is obtained from two directions at right angles to each other hereinafter.
4. Referring to analysis of specimens, upper analysis refers to that of hot rolled silicon steel stock while the lower to that of prior to final anneal.
5. Each specimen consists of the above composition and the balance, iron and incidental impurities, described hereinbefore.

It will be easily understood from the analytical data for hot-rolled sheets, which are identical with those for the sheets prior to the final anneal, in Table 1, that the content of acid-insoluble Al is almost constant, i.e., in the order of 0.005%, independently of the total amount of Al. It will also be easily understood that the amount of acid-soluble Al changes in proportion to the amount of total Al so that more than 60% of the total amount of aluminum present exists as acid-soluble Al and a substantial portion of the latter as AlN. In other words, in the case of using no special melting apparatus which removes nitrogen from the treated steel, the acid-soluble Al in the produced hot-rolled sheets consists to a substantial portion, preferably one-third, of AlN.

Referring again to Table 1 and FIGURE 4, while in the case of starting materials A and E, the magnetic properties after final anneal are ordinary, for example, the magnetic induction  $B_{10}$  is less than 17,000 gauss in each product, in the case of the starting materials B, C and D, the magnetic induction  $B_{10}$  in each product is about 18,000 gauss in both outstanding directions, namely the direction of final rolling and the direction perpendicular thereto, and the products thus show the outstanding properties of double oriented silicon steel.

The values (Epstein test) of magnetic induction  $B_{10}$  in the rolling direction of top-class products by three steel manufacturers which have been marketed heretofore as single oriented silicon steel are as follows by the catalogs of the manufacturers:

| Name of Firm            | Trade Name of Product      | Thickness     | $B_{10}$ (gausses) |
|-------------------------|----------------------------|---------------|--------------------|
| Yawata Iron & Steel Co. | Orient Cor Z11.....        | 0.35 mm.....  | 17,800             |
| Armeo.....              | M 6 X.....                 | 0.014 in..... | 17,600             |
| U.S. Steel Co.....      | U.S.S. Transformer 66 M-6. | 0.014 in..... | 18,000             |

As the value of  $B_{10}$  is a value of a magnetic induction in a magnetic field of 10 oersteds, the higher this value is, the better the parallel relation between the easy magnetization axis, i.e., the [100] axis and the rolling direction. The value of  $B_{10}$  in an oriented silicon steel sheet is usually higher than 17,000 gauss. Since, moreover, in single oriented silicon steel, an easy magnetization axis does not appear in the direction perpendicular to the rolling direction as shown in FIG. 1(a), the value of  $B_{10}$  in the said transverse direction is far lower. On the other hand, in the products of this invention obtained from the starting materials A, C and D, the values are about 18,000 gauss in both directions, which proves that the product in this invention is clearly double-oriented silicon steel of the type illustrated in FIG. 1(b). Thus, we have found by comparing and investigating the relations between Al contents after hot rolling and magnetic inductions of products, that, contrary to the teaching of the most recent known process (U.S. Patent 3,008,856), the Al content after hot rolling must be restricted to the range between 0.010 and 0.040% in the case of the treatment by the aforesaid process mode A. In particular, when the Al content is in a range of 0.015 to 0.030%, the magnetic induction  $B_{10}$  of the final product is higher than 18,000 gauss in the direction of the final rolling, as well as in the direction perpendicular thereto, which values are even better than the best values of magnetic induction  $B_{10}$  of a conventional single oriented silicon steel in the rolling direction.

The thickness or gauge of the hot rolled steel is an important requirement for the production of a doubly oriented silicon steel sheet or strip. In our process mode A, the thickness or gauge of the starting material should be preferably 2.5 to 10 times of the desired final thickness or gauge.

If the gauge of the hot rolled silicon steel is too thin, the hot rolling procedure will be very difficult to carry out. On the other hand, if the gauge of the hot rolled

silicon steel is too thick, the final gauge of the product will be too thick after the predetermined cold rolling reduction, which results in an increase of eddy loss.

In view of the above requirements, the gauge of the hot rolled silicon steel is preferred to be from 1 mm. to 4 mm. Particularly, about 1.6 mm. is most preferred, which is about three to five times the final gauge, taking both the final and the necessary cold rolling into account.

The hot rolled silicon steel with a predetermined gauge is subjected to a pickling step, and then to cold rolling.

The reduction in thickness by cold rolling is of the greatest importance in view of the combination of two cold rolling directions. In one embodiment of the invention, the overall reduction is preferred to be within the range of 60% to 90%. The embodiment which comprises cold rolling the steel in one direction first with a reduction of 40% to 80%, again cold rolling it in another direction at right angle thereto, with a reduction of 30% to 70%, and finally annealing the thus cold rolled steel, has resulted in the desired cube oriented silicon steel sheet or strip we have in view.

It is most preferred to take the combination of two cold rolling steps consisting of the initial cold rolling in one direction with a reduction of about 60% and the

final cold rolling in a crosswise direction thereto (at an angle of about 90%) with a reduction of about 50%. When the direction of the initial cold rolling step coincides with or deviates at a certain angle from that of hot rolling the starting material, we have found that the iron core

loss and magnetic induction determined after the final anneal in reference to the one direction of initial cold rolling are not appreciably different from those obtained from the other direction of final cold rolling. It is important, in order to obtain good results in the process of the invention, that the two directions of cold rolling are approximately at right angles to each other. The more the angle deviates from the right angle, the more difficult will it be to obtain a product favored with two axes of easy magnetization [001]. In view of the above consideration, we have discovered that a permissible angle crossing to each other should deviate less than  $\pm 20^\circ$ , and, to obtain good results, not more than  $\pm 15^\circ$ , from the direction of the right angle.

In a commercial production embodying the process of our invention, the hot rolled silicon steel containing more than 2.5 and up to 4% of silicon and between 0.010% and 0.040% aluminum is cold rolled in one direction, then sheared off to a sheet of length, and again cold rolled in the other direction at right angle  $\pm 15^\circ$  thereto in the form of sheet. Alternatively, another silicon steel strip is produced by welding sheared sheets end to end together in such manner that the longitudinal direction of the strip makes a direction at right angle, or deviating by less than  $15^\circ$  therefrom on either side, to the direction of initial cold rolling, whereupon the strip is again cold rolled continuously.

The welding operation of sheets to strip makes no difference for the advantage of the invention, even though it may be carried out at any step after the initial cold rolling procedure.

A preferred commercial production carrying out the process of the invention with the hot rolled silicon steel strip as starting material comprises the following steps:

A hot rolled silicon steel strip having a predetermined thickness is pickled to remove scale resulting from hot rolling with the above-defined definite reduction to produce cold rolled silicon strip. The cold rolled silicon strip is sheared off to a number of sheets of desired length. Subsequently, a new silicon steel strip is produced by welding the sheared length of sheets end to end together in such a manner that the longitudinal direction of the new strip forms a direction at right angle or deviating less than  $\pm 15^\circ$  therefrom, to the direction initial cold rolling, then the thus produced strip is again cold rolled continuously with a predetermined reduction. Alternatively,

a sheared length of sheet is again cold rolled sheet by sheet in a direction at right angle or deviating less than  $\pm 15^\circ$  from the direction of initial cold rolling, with a predetermined reduction, then a number of twice cold-rolled sheets are welded end to end together to produce a new cold rolled strip. Of course, the above-described subsequent treatment will be given to the cold-rolled strip thus obtained.

The temperature of the short time anneal to be imparted to the silicon steel sheet or strip which has been cold rolled to the final gauge has an influential effect on the primary recrystallization structure resulting from the anneal, and the secondary recrystallization of the seed crystal grain having a (100)[001] type orientation will depend upon the primary recrystallization structure.

FIGURE 6 shows the influence of the annealing temperature on the iron core loss after the final anneal of a product which has been obtained by the process of the invention wherein a hot-rolled silicon steel containing 0.03% carbon, 3.02% silicon, 0.018% aluminum in all, and 0.013% acid-soluble aluminum with a gauge of 1.75 mm. was first cold-rolled in one direction with a reduction of 60%, and then again cold rolled to final gauge in another direction approximately at right angles to the direction of the first cold rolling, with a reduction of 50%, and then annealed for four minutes at a temperature ranging between 700° and 1,200° C. It is clear from FIGURE 6 that the temperature at which a short time anneal should be carried out is preferably a temperature between 750° and 1,000° C., in order to obtain a product having good magnetic properties, while at a higher temperature than the above upper limit, even for a short period of time only, the grain growth of primary recrystallization structure may become so considerable that selective secondary recrystallization in the final anneal will be prevented, although the advantage of the present invention may not be entirely lost. Further, it is to be understood that the advantage of the invention will not be lost as long as the temperature of the short time anneal is within the range between less than 750° C. and higher than the recrystallization temperature. However, the temperature ranging between 750° and 1,000° C. specified hereinabove is preferred for production on an industrial scale, since the lower temperature takes a longer, and therefore uneconomical, time towards attaining the completely recrystallized structure. The time required for anneal at the above temperature range takes usually about one minute for the cold rolled structure of the steel to be converted into the recrystallized structure. Since the silicon steel stock contains approximately 0.04% carbon, decarburization is required at the same time to an extent at which crystal growth may not be interfered with by the presence of carbon in the final anneal. We have discovered that a maximum of up to four minutes is required

for continuous anneal in view of the thickness of the material and other requirements. It is to be understood, however, that the period of time for the short time anneal should not limit the present invention. This anneal is carried out usually in a neutral or reducing atmosphere, but is not necessarily limited thereto. Further, it is considered that the temperature ranging between 750° and 1,000° C. specified above is beneficial to commercial production because a decarburizing reaction is most actively going on at the above temperature in the presence of a small amount of moisture. A silicon steel sheet or strip which has been annealed for a short period of time may be subjected to pickling depending on its surface conditions.

Referring to the last anneal, an anneal at a temperature above 900° C. in the reducing atmosphere for a period of time more than at least five hours is required in order to produce a cube-oriented silicon steel strip having low core loss and high magnetic induction values. The complete secondary recrystallization may not be developed by an anneal at either lower temperature or shorter time than that defined above. A practical temperature available for the commercial production of the invention is preferred to be between 900° and 1,300° C., since an anneal at either a temperature above 1,300° C. or for a time longer than forty hours is not so effective. Annealing at a temperature outside the range described above, however, will not lose the fundamental advantage of our invention.

By the improved process according to the invention, it becomes possible, for the first time, to obtain uniform results of double orientation steel made with conventional apparatus available in industry.

#### PROCESS MODE B

In the following Table 2 there are compiled data obtained by applying above-mentioned mode B of carrying out the process of the invention to hot-rolled sheets or strips of 2 mm. thickness, which are produced by subjecting to a conventional hot-rolling process the ingots produced, in turn, by a conventional open-hearth steel-making process; the hot-rolled ingots are cold-rolled to a direction which is identical with the hot-rolling direction, at a reduction rate of about 30%, then cold-rolled in the direction perpendicular to the first cold-rolling direction at a reduction rate of approximately 30%, thereafter annealed for 5 hours at a maximum temperature maintained at 1100° C., cold-rolled again at a reduction rate of 70% in a direction coincident with the last-preceding rolling direction in the aforesaid cross rolling, and then finally annealed for 15 hours at 1150° C.

In FIG. 5 there are shown the relations between the Al contents in the hot-rolled sheets and the iron loss values and magnetic induction values of the final-annealed sheets.

Table 2

ANALYSIS OF STEEL AND MAGNETIC PROPERTY

| Sample | Analysis (Percent) |      |          |              |         |          | Mag. test (Epstein)  |                            |
|--------|--------------------|------|----------|--------------|---------|----------|----------------------|----------------------------|
|        | C                  | Si   | Total Al | Acid-sol. Al | Total N | N as AlN | Iron loss            | Magnetic Induction         |
|        |                    |      |          |              |         |          | W <sub>15/50</sub>   | B <sub>10</sub>            |
| A'     | 0.04               | 3.05 | 0.005    | 0.002        | 0.0035  | 0.0005   | 1.90<br>1.87<br>1.87 | 15,200<br>15,250<br>15,250 |
| B'     | 0.04               | 3.01 | 0.015    | 0.010        | 0.0045  | 0.0029   | 1.42<br>1.42<br>1.40 | 17,150<br>17,150<br>17,400 |
| C'     | 0.04               | 3.11 | 0.021    | 0.016        | 0.0049  | 0.0045   | 1.04<br>1.04<br>1.09 | 18,050<br>18,050<br>17,950 |
| D'     | 0.04               | 3.02 | 0.026    | 0.020        | 0.0060  | 0.0059   | 0.99<br>1.01<br>1.01 | 18,250<br>18,150<br>18,150 |
| E'     | 0.04               | 3.06 | 0.041    | 0.032        | 0.0078  | 0.0073   | 1.19<br>1.26<br>1.26 | 17,800<br>17,700<br>17,700 |
| F'     | 0.04               | 3.01 | 0.065    | 0.051        | 0.0080  | 0.0070   | 1.47<br>1.47<br>1.55 | 17,100<br>17,100<br>17,000 |

Notes:

1. W<sub>15/50</sub> means an iron core loss at 15,000 gauss measured per frequency of 50, and its unit is w./kg.
2. B<sub>10</sub> means a magnetic induction at 10 oersteds, and its unit is gauss.
3. In reference to the magnetic property, the upper one is the value measured along the final rolling direction and the lower is that along the direction at a right angle thereto.

As clearly indicated in Table 2, good orientations in two directions of cold rolling and a low core loss are given to the hot rolled silicon steel material after the final anneal while, on the contrary, similar results are not obtained by the conventional silicon steel containing either less than 0.010% Al or more than 0.050% Al despite of the same treatment.

From the analytical data after hot rolling shown in Table 2, it can be seen that the amount of acid-insoluble Al remains almost constant independently of the total amount of Al, and acid-soluble Al mainly consists of AlN, which data are very similar to the analytical data after hot rolling stated in process A, *supra*.

Referring now to Table 2 and FIGURE 5 more in detail, while in the case of starting material A', the magnetic properties after final anneal are low, for example, the magnetic induction  $B_{10}$  is less than 17,000 gauss, in the case of the products obtained starting materials B', C', D', E' and F', the magnetic induction  $B_{10}$  of each product is about 18,000 gauss in the two outstanding directions, i.e., the direction of final rolling and the direction perpendicular thereto, which shows that the products are indeed, improved double-oriented silicon steels. We have found that the content of Al must be limited to the range between 0.010 and 0.050% in the case of the treatment by process mode B. We have further found that, while even in the case of material F' containing 0.065% of Al, the magnetic induction  $B_{10}$  of the final product is higher than 17,000 gauss, yet, as the content of Al is more than 0.050%, the amount of acid-insoluble Al increases, as already stated, which influences the iron loss and other magnetic properties in an undesirable manner. Therefore, the Al content is in a range of 0.020 to 0.035%, the magnetic induction  $B_{10}$  of the final product is higher than 18,000 gauss in the direction of final rolling and the direction perpendicular thereto, which is an excellent increase above the value of magnetic induction  $B_{10}$  which a conventional single-oriented silicon steel shows in the rolling direction.

Now, each of the processing steps for carrying out the mode B of the process according to the invention will be described. As has been mentioned before, the gauge or thickness of hot rolled steel is an important factor in order to manufacture a double-oriented silicon steel sheet or strip we have in view. In the case of mode B, the gauge of the hot-rolled silicon steel starting material should be preferably 5 to 30 times as thick as the final desired gauge. This gauge is closely related to the total reduction of cold rolling described hereinbelow, an excessively thin gauge of the hot-rolled material leading to the same difficulties as described under Process mode A, and, conversely, an extremely thick gauge thereof resulting in a thick gauge of the final product obtained by the reduction required for cold rolling, which will also result in an undesirable increase of eddy current loss due to the thick gauge.

Accordingly, the gauge of the starting material is usually preferred to be from 0.7 to 13 mm., and particularly, about 3 mm. gauge of the starting material is desired taking both the final gauge and the necessary cold rolling reduction into account.

The hot rolled silicon steel is pickled in the usual manner in order to remove scale resulting from hot rolling. The reduction in thickness by cold rolling carried out after pickling in two stages in directions at right angle to each other is of utmost importance depending on the combination of rolling directions. In this mode B, an overall reduction of 44-80% is preferred: the primary cold rolling reduction in one direction should be 30-60%, and the secondary cold rolling reduction in the other direction at a right angle thereto 20-50%. When the most desirable gauge, 3 mm., of the above hot rolled steel is adopted, the combination of a cold rolling reduction of 40% in one direction and a second reduction of 40% in the other direction at right angle thereto is preferable.

Two types of the final product are obtained by the process of this invention: one is obtained by the process which involves a direction of primary cold rolling coinciding with that of the preceding hot rolling, and the other is obtained by the process which involves a direction of primary cold rolling being at a certain angle to that of hot rolling. When these two products are compared, hardly any appreciable difference is perceived between iron core losses and magnetic inductions determined along the two directions, respectively, after the final anneal. However, considerable attention should be paid to the fact that the degree of an angle at which the secondary cold rolling is carried out relative to the direction of the primary cold rolling has a significant influence on the magnetic properties of the product after the final anneal. In accordance with the present invention, approximately 90° is the most preferred angle between the primary and secondary rolling directions. The more this angle deviates, the more difficult is it to develop the axis of easy magnetization [001] in the two directions. We have found that the desired doubly-oriented silicon steel sheet or strip could not be obtained, if the deviation from the right angle amounts to 15° or more. Therefore, the permissible degree of deviation of the crossing angle from 90° is within the range of  $\pm 15^\circ$  in mode B as well as in mode A of carrying out the process of our invention.

We employ, for instance, a hot rolled steel strip as silicon steel starting material. When this steel material in strip form is subjected to the required process of the invention, the silicon steel strip having a predetermined gauge is first pickled to remove hot rolling scale, then cold rolled with the necessary reduction to obtain a cold rolled steel strip, which is cut into a number of sheets of a predetermined length, two or more sheets are welded together end to end in order to make a new steel strip the longitudinal direction of which is in a direction at an angle of approximately 90° (with a deviation within the range of  $\pm 15^\circ$ ) to the direction of the primary cold rolling, whereupon the welded strip is subjected to the secondary cold rolling, further followed by the subsequent treatment described further below.

In case of a steel strip as a starting material in this invention, there are several processing methods to be considered as follows:

- (1) A first cold rolling is applied to the steel in the form of a strip, and the subsequent processing steps are applied to it in the form of a sheet;
- (2) A first cold rolling is applied to a steel strip which is then cut into a number of sheets of a predetermined length, then a second cold rolling is applied to the steel in the form of a sheet in a direction at an angle of 90° (with a deviation within the range of  $\pm 15^\circ$ ) to the direction of the first cold rolling, then two or more of such twice cold rolled sheets are welded together end to end to form a new strip whose longitudinal direction is equal to either one of the two directions of cold rolling, and thereafter the subsequent processing steps described further below are applied to this new strip;
- (3) A first cold rolling is applied to a steel strip, which is then cut into a number of sheets of predetermined length, then a second cold rolling and an intermediate box anneal (described hereinafter) are applied to the steel in the form of a sheet under the required conditions, then two or more sheets are welded together end to end to form a new strip whose longitudinal direction is equal to either of the two directions of cold rolling, and thereafter the subsequent processing steps are applied to the new strip; and
- (4) A first cold rolling is applied to the steel in the form of a strip, which is then cut into a number of sheets of predetermined length, then a second cold rolling, an intermediate box anneal and a final cold rolling, described further below, are applied to the steel in the form of a sheet under the required conditions, then two or more

sheets are welded end to end together to form a new strip whose longitudinal direction is equal to either of the two directions of cold rolling, and thereafter the subsequent processing steps are applied to this new strip.

When a hot-rolled steel sheet is used as starting material, there are also several processing methods to be considered as follows:

(1) A first cold rolling is applied to a steel sheet in one direction, then this steel sheet is cut into sheets of a predetermined length, then two or more sheets of this length are welded together end to end to form a new steel strip whose longitudinal direction is at an angle of 90° (with a deviation within the range of  $\pm 15^\circ$ ) to the direction of the first cold rolling, and thereafter the second cold rolling and subsequent processing steps are applied to this new steel strip;

(2) Two cold rolling steps in two crossing directions are applied to the steel in the form of a sheet, then two such sheets are welded together end to end to form a new strip whose longitudinal direction is the same as either of the two crossing directions, and thereafter the subsequent processing steps are applied to this new strip;

(3) Two cold rolling steps in two directions and an intermediate box anneal (described hereinafter) are applied to a sheet, then two or more of such sheets are welded together end to end into a new strip whose longitudinal direction coincides with one of the two crossing directions, and thereafter the subsequent processing steps are applied to this new strip; and

(4) A series of the required steps up to the final cold rolling (described further below) is applied to the steel in the form of a sheet, then two or more sheets are welded end to end together to form a steel strip, and thereafter the subsequent processing steps are applied to this strip. It is to be understood that the above described welding operation is not always necessary.

An intermediate box anneal imparted to the silicon steel sheet or strip reduced in thickness to an intermediate gauge by two cold rolling steps in two mutually crossing directions has an important influence on the recrystallized structure to be produced by subsequent annealing. In this invention, the maximum holding temperature range should be preferably from 850° to 1200° C. during the intermediate box anneal.

FIG. 7 is a graph showing the effect of the temperature of the intermediate box anneal on the magnetic properties of a magnetic material produced by the process of this invention, wherein a hot rolled silicon steel containing 3.02% Si, and 0.026% Al was subjected to a first cold rolling with a reduction of about 30% in the same direction as that of hot rolling, then again to a second cold rolling with a reduction of about 30% in a direction approximately at right angles thereto, then to anneal for a period of 5 hours at a temperature if 800° to 1200° C. as the maximum holding temperature, then again to a final cold rolling with a reduction of 70% in the same direction as that of the second cold rolling, and lastly to a final anneal for a period of 15 hours at a temperature of 1150° C.

It is clear from FIG. 7 that the higher the maximum holding temperature, the more effective the anneal, but FIG. 7 also shows that this effect changes very little at temperatures above 1000° C. However, the magnetic properties will decrease at temperatures below 850° C. Accordingly, from a commercial point of view, we prefer the maximum holding temperature range for the intermediate box anneal to be 850° to 1200° C. An atmosphere of either neutral or reducing gas medium is usually employed, but we do not limit the process of our invention thereto. Sufficient nitrogen should, of course, be present in this medium.

The reduction in thickness of the final cold rolling procedure is an important factor for attaining the double-oriented silicon steel we have in view, and the direction at which this final cold rolling is carried out should be a

5

direction approximately equal to either of two crosswise directions of the preceding two cold rolling stages. From a commercial point of view, the selection of the same direction as that of the second cold rolling is most practical.

FIG. 8 is a graph showing the relationship between the magnetic induction and the cold rolling reduction of a magnetic material manufactured by the process of the invention wherein a hot rolled silicon steel material of 3.0 mm. thickness and containing 3.05% Si and 0.034% Al was subjected to a first cold rolling, with a reduction of 40%, in the same direction as that of hot rolling, then again to a second cold rolling in a direction approximately at right angle thereto with a reduction of 40%, then to an anneal for a period of 5 hours at a temperature of 1100° C., the maximum holding temperature, then to a final cold rolling in the same direction as that of the second cold rolling with a reduction ranging from 19 to 84%, and lastly to a final anneal for a period of 15 hours at a temperature of 1150° C. The foregoing results show that the reduction in thickness by the third or final cold rolling procedure is preferably within the range of 50 to 84%, and more particularly, a reduction of approximately 70% is most desirable.

As mentioned above, the silicon steel sheet reduced in thickness to the final gauge by the foregoing processing steps is subjected to a final anneal. With a view to attaining a double-oriented silicon steel strip having a low iron core loss, it is required to anneal the steel for a period of more than 5 hours at the maximum holding temperature of above 1000° C. in a neutral or reducing atmosphere. By an anneal at a lower temperature than the above, a complete growth of crystal cannot be developed. Conversely, an anneal either at an elevated temperature of above 1300° C. or for an extended period of more than 40 hours will not develop the desired effect in a satisfactory manner despite of the elevated temperature or the extended anneal time. Accordingly, we prefer a temperature range of 1000° to 1300° C. as the best commercially effective anneal. However, the fundamental effect of the present invention will not be lost completely by an anneal deviating from the range of either temperature or period of time mentioned above.

The desired double oriented silicon steel sheet or strip can be manufactured in accordance with the complete process of this invention described hereinabove. It is to be understood that the carbon content of the product after the final anneal should be the least possible, and more particularly, a content of less than 0.005% C is most desirable.

Silicon steel used as starting material in carrying out the process of invention may usually contain 0.02-0.06% C. Therefore, a decarburizing anneal should be effected in order to reduce the carbon content, provided that it has not been reduced as desired by the intermediate and final box anneals. To this end, various known processes of anneal may be applied in practicing our invention, and we do not intend to limit ourselves to a particular one. For example, decarburization can be achieved by a process which comprises subjecting a hot rolled material with scale thereon to a box anneal, and also by a process which comprises subjecting a steel material either after two cross cold rolling steps or after the final cold rolling step to a short time anneal in an atmosphere containing either neutral or reducing gas and a small amount of moisture. We have discovered that the carbon content of the final product can be easily reduced to less than 0.005% by means of either of the above two processes of decarburization or by both combined.

We therefore, recommend that a box anneal with scale at a temperature of 650°-900° C., and a short time anneal in an atmosphere containing a little moisture at a temperature at 750°-950° C. be effected in the process of our invention.

At first glance, it may seem that the number of steps in the process mode B is, as stated above, more than that of

60

65

70

75

the process mode A and consequently that the process mode B is not as economical as the process mode A. However, as the permissible range of Al content for imparting the magnetic properties of double oriented silicon steel (according to a commonly applied standard B<sub>10</sub> of the silicon steel must be higher than 17,000 gauss in a rolling direction and a direction perpendicular thereto), is broader in process mode B, the latter is less subjected to the troubles which may be caused by the segregation of Al in the material. Also, the magnetic properties of the product obtained from a material containing the most suitable amount of Al by the process mode B are somewhat better than those of the product obtained by the process mode A.

Our invention is further illustrated but not limited by the following examples:

*Example 1*

Hot rolled silicon steel stock containing 0.04% C, 2.98% Si, a total content of 0.019% Al, comprising 0.015% acid-soluble Al and 0.0061% of AlN, and having a thickness of 1.6 mm., was pickled, cold rolled with a reduction of 60% in one direction, then again cold rolled with a reduction of 50% in another direction approximately at right angle thereto to a final gauge of about 0.33 mm. thickness. The thus treated silicon steel was subjected to a continuous anneal for four minutes at the temperature of 800° C. in order to decarburize and recrystallize it, and to a final box anneal for 15 hours at the temperature of 1150° C., to develop the magnetic properties thereof. Magnetic tests according to Epstein were conducted on a sample taken from the above material with regard to the direction of the final cold rolling and also the direction at right angle thereto after the stress relief anneal, the results of which test are shown in the respective columns of Sample C of Table 1 as magnetic induction and iron core loss. As illustrated in FIG. 9, the magnetic torque curve diagram of this product shows that it is favored with an excellent structure of cube orientation.

*Example 2*

Hot rolled silicon steel strip containing 0.04% C, 2.99% Si, a total content of 0.023% Al comprising 0.018% acid-soluble Al and 0.0061% AlN, and having a thickness of 1.6 mm., was pickled, cold rolled with a reduction of 60% in the same direction as that of the preceding hot rolling to produce a cold rolled silicon steel strip of 0.64 mm. thickness. Subsequently, the silicon steel strip was sheared off to a number of sheets of definite length, which were welded together sheet by sheet in order to produce a new silicon steel strip whose longitudinal direction was approximately at right angle to the direction of the initial cold rolling. The new silicon steel strip was again cold rolled with a reduction of about 50% to a thickness of 0.33 mm. The cold rolled strip was subjected to a continuous anneal for four minutes at a temperature of 800° C. followed by a box anneal for 15 hours at a temperature of 1150° C. Magnetic tests were conducted on an Epstein test sample taken from the above magnetic material with regard to its longitudinal direction and also to the direction approximately at right angle thereto, after the stress relief anneal, the results of which tests are shown in the respective columns of Sample D of Table 1 as magnetic induction and iron core loss.

*Example 3*

A hot rolled silicon steel material of 2 mm. thickness, containing 0.04% C, 3.06% Si and 0.030% Al (comprising 0.024% of acid-soluble Al, and 0.0069% of AlN) is cold rolled with reduction of 30% in one direction, then again cold rolled with a reduction of 30% in another direction displaced approximately at a right angle to the first rolling direction to an intermediate gauge of 0.98 mm., and annealed for a period of 10 hours at the maximum holding temperature of 950° C.

Thereafter, this steel is further cold rolled with a reduction of 68% in the same direction as that of the second cold rolling step described above to a final gauge of 0.31 mm., and then finally box-annealed for a period of 20 hours at a maximum holding temperature of 1200° C. to develop the magnetic properties thereof.

From this product, Epstein samples are taken along the final rolling direction and also along the direction displaced at a right angle thereto, respectively, and magnetic tests are conducted on them after the stress relieving anneal, the results of which are as follows:

|                              | B <sub>10</sub><br>(gauss) | W <sub>15/50</sub><br>(w./kg.) |
|------------------------------|----------------------------|--------------------------------|
| 15                           |                            |                                |
| Final Rolling Direction..... | 17,800                     | 1.26                           |
| Right Angle Direction.....   | 17,650                     | 1.34                           |

The above values indicate an excellent cube structure.

*Example 4*

The same hot rolled silicon steel material as in Example 3 with scale thereon is box-annealed for a period of 5 hours at a temperature of 680° C., then cold rolled with a reduction of 30% in one direction, then again cold rolled with a reduction of 30% in another direction displaced approximately at a right angle the first direction of rolling to an intermediate gauge of 0.98 mm., and box-annealed for a period of 5 hours at a maximum holding temperature of 1100° C.

Thereafter, this steel is further cold rolled with a reduction of 70% in the same direction as that of the second cold rolling step described to a final gauge of 0.30 mm., and finally box-annealed for a period of 15 hours at a maximum holding temperature of 1150° C. to develop the magnetic properties thereof.

From this product, Epstein samples are taken along the final rolling direction and also along the direction displaced at a right angle thereto, respectively, and magnetic tests are conducted on them after the stress relieving anneal, the results of which are as follows:

|                              | B <sub>10</sub><br>(gauss) | W <sub>15/50</sub><br>(w./kg.) |
|------------------------------|----------------------------|--------------------------------|
| 45                           |                            |                                |
| Final Rolling Direction..... | 18,250                     | 0.99                           |
| Right Angle Direction.....   | 18,050                     | 1.04                           |

The above indicates an excellent cube structure.

*Example 5*

A hot rolled silicon steel material of 3.0 mm. thickness, and containing 0.04% C, 3.05% Si and a total content of 0.034% Al (comprising 0.029% of acid-soluble Al and 0.0072% of AlN) is cold-rolled in the same direction as that of hot rolling, to a cold rolled silicon steel strip of 1.8 mm. thickness. Thereafter this strip is cut into a number of sheets of a predetermined length, which sheets are welded together end to end to form a strip whose longitudinal direction is displaced at a right angle to the direction of the first cold rolling. This new strip is cold rolled with a reduction of 40% to an intermediate gauge of 1.08 mm. It is then annealed at a maximum holding temperature of 1100° C. for a period of 10 hours, then again cold rolled with a reduction of 72% in the direction of its longitudinal length to the final gauge, then annealed at a temperature of 800° C. for a period of 3 minutes in a wet hydrogen atmosphere to decarburize it, and finally box-annealed at a maximum holding temperature of 1200° C. for a period of 20 hours in order to develop its magnetic properties. From this product, Epstein samples are taken along its longitudinal direction and also along a direction displaced at a right angle thereto, respectively, and magnetic tests are conducted on

the samples after the stress relieving anneal, the results of which are as follows:

|                             | B <sub>10</sub><br>(gauss) | W <sub>10/60</sub><br>(w./kg.) |
|-----------------------------|----------------------------|--------------------------------|
| Longitudinal Direction..... | 18,340                     | 0.98                           |
| Right Angle Direction.....  | 18,150                     | 1.05                           |

The above values show that a double-oriented silicon steel strip with a good cube structure has been manufactured.

We claim:

1. A process for producing double-oriented silicon steel sheet having (100)[001] crystal orientation and good magnetic properties in the final-rolling direction and the direction perpendicular thereto, which comprises
  - (a) pickling a hot-rolled silicon steel material consisting essentially of iron, from 2.5 to 4.0% by weight Si, and from 0.010 to 0.040% by weight Al, a substantial portion of said Al being in acid-soluble form which consists essentially of aluminum nitride,
  - (b) cold rolling said material in one direction at a reduction rate of from about 40 to 80%,
  - (c) cross cold rolling the resulting material in a direction at an angle from 90° to an angle deviating from 90° by less than ±15°, with the direction of said first cold rolling and at a reduction rate of from about 30 to 70%,
  - (d) annealing the resulting cross-rolled material for about one to four minutes at a temperature from 750 to 1000° C. to effect decarburization and primary recrystallization, and
  - (e) finally annealing the material for about 5 to 40 hours at a temperature of about 900° to 1300° C.,

thereby obtaining a double oriented silicon steel with (100)[001] type crystal orientation and

outstanding magnetic properties in the aforesaid two directions.

2. A process for producing double-oriented silicon steel having (100)[001] crystal orientation and good magnetic properties in the final-rolling direction and the direction perpendicular thereto, which comprises

- (a) pickling a hot-rolled silicon steel material consisting essentially of iron, from 2.98 to 3.11% by weight of Si, and from 0.016 to 0.030% by weight of Al, a substantial portion of said Al being in acid-soluble form which consists essentially of 0.0029%–0.0073% by weight, based on the hot-rolled silicon steel, of aluminum nitride,
- (b) cold rolling said material in one direction at a reduction rate of from about 40 to 80%,
- (c) cross cold rolling the resulting material in a direction at an angle from 90° to an angle deviating from 90° by less than ±15°, with the direction of said first cold rolling and at a reduction rate of from about 30 to 70%,
- (d) annealing the resulting cross-rolled material at a temperature of from 750 to 1000° C. to effect decarburization and primary recrystallization, and
- (e) finally annealing the material for about 5 to 40 hours at a temperature of about 900 to 1300° C., thereby obtaining a double-oriented silicon steel with (100)[001] type crystal orientation, the magnetic induction of which, in the said two directions and in a magnetic field of 10 oersted, exceeds 18,000 gauss.

References Cited in the file of this patent

UNITED STATES PATENTS

- |           |            |                |
|-----------|------------|----------------|
| 2,173,240 | Wassermann | Sept. 19, 1939 |
| 2,867,557 | Crede      | Jan. 6, 1959   |
| 2,965,526 | Wiener     | Dec. 20, 1960  |
| 3,008,856 | Mobius     | Nov. 14, 1961  |